

Jan. 5, 1960

C. J. HECHINGER

METAL FABRICATION

2,919,471

Filed April 24, 1958



INVENTOR:

CARL J. HECHINGER

By *Lincoln S. Hoff* and *Robert F. Kuemel*  
ATTORNEYS.

## 1

2,919,471

## METAL FABRICATION

Carl J. Hechinger, St. Louis, Mo., assignor to Olin Mathieson Chemical Corporation, East Alton, Ill., a corporation of Virginia

Application April 24, 1958, Serial No. 732,112

17 Claims. (Cl. 18—47.2)

This invention relates to pellets and more specifically to a method for treating metal and making metal pellets, and is a continuation-in-part of application Serial Number 562,447, now abandoned, filed January 31, 1956.

In certain fabricating operations, particularly in the extrusion of metal parts, slugs of metal are fed into a machine and fabricated into useful articles. These slugs must be of substantially uniform weight, size, shape and composition. Heretofore such slugs have usually been either stamped from sheets, cut from bars or individually cast in molds. Although slugs formed in this manner are satisfactory, it is of course highly desirable that the cost of producing the slugs be reduced to the greatest degree possible.

In the manufacture of metal pellets, such as lead pellets, it has been the general practice to drop globules of molten metal through a cooling medium such as a 100 foot column of air, a water spray, or steam, and to catch the solidified globules in water which may be provided with additives for cleaning the pellets or for applying a protective coating to the pellets. It is during this fall that the globule solidifies with the result that upon striking the water bath in the base of the tower the globule is substantially solid. When the 100 foot column of cooling gas or vapor is reduced and the globule strikes the water bath after a fall of only a few feet the resultant pellets are not spherical. At best they have shrink holes and usually they splatter into an irregular mass resembling popped popcorn. This method of fabricating pellets has given rise to the familiar tall and slender dropping tower having a height of about 100 to 150 feet through which the globules are dropped into a deep well. The dropping tower process is the most widely used method of fabricating pellets of lead for use in sporting ammunition. Unfortunately only a few metals such as lead can be satisfactorily fabricated into pellets by this method.

Other methods of forming pellets are known such as, dropping globules of molten metal through a relatively short column of air and into various solutions such as a bath of water in which is dissolved soluble alcohol, ketones, aldehydes, esters of organic acids or water solutions containing fluxes such as zinc chloride or ammonium chloride. Many metal pellets made by these methods tend to develop gas pockets or splatter upon contact with the liquid bath. This is particularly true in the fabrication of aluminum, nickel or copper pellets. Another previously known method of fabricating pellets comprehends dropping molten metal into pulverized graphite. When this method was tried it was found that the pellets would tend to flatten out, that the surface of the pellets was rough and contaminated by the graphite. The dropping of the globules of metal into water and liquid solutions, single-phase, was proven unsatisfactory when

## 2

the surface of the pellets was also found to be rough and the pellets misshapen. Still another previously known method of fabricating pellets involves dropping molten metal into a liquid bath which is relatively cool in its lower regions and hot in its upper regions so that the pellet passed through the hottest portion of the bath and into the cooler portion. The temperature differential of the quenching bath did not appear to have any substantial advantages.

- 5 10 15 20 25
- It has also been proposed to form pellets by eliminating any free drop and passing molten metal globules directly into a cooling bath of another molten metal having a melting point below the solidification temperature of the molten globules and relying on the difference in density between the metals to cause the globules to pass through the cooling medium. None of these methods produce satisfactory pellets either because the size of the resultant pellets is too small or cannot be controlled accurately, or because the resultant pellets contain gas pockets or are in the form of a splattered mass of metal resembling popped popcorn rather than substantially spherical pellets.

Certain of the above described methods, particularly the dropping tower method, will produce pellets of sufficiently large size and consistent configuration for use in some shot gun shells and similar applications. However, such a process does not lend itself to the production of larger pellets and the dropping tower method has the obvious additional disadvantage of requiring a location where such a structure may be erected and these structures are expensive to build.

It is therefore an object of this invention to produce by a dropping process, metal pellets having a practicable size and consistency for use in subsequent metal fabricating processes.

Another object of this invention is to fabricate by a dropping process metal pellets of relatively large and consistent size.

Another object of this invention is to fabricate by a dropping method pellets having a generally spherical configuration.

Another object of this invention is to provide a novel method for subdividing a mass of metal into spherical pellets.

45 40 45 50 55

Another object of this invention is to provide pellets which are not unduly porous and which have a relatively smooth surface.

Another object of this invention is to provide a method of producing pellets in a relatively limited space and with apparatus having a small initial cost.

Another object of the invention is to produce metal pellets more safely.

Additional objects and advantages will become apparent from the following description and drawings in which:

55 50 55

Figure 1 is a schematic sectional view illustrating one method of obtaining the correct dropping temperature of the metal, and

Figure 2 is a schematic sectional view illustrating an embodiment of a suitable pellet making apparatus in operation.

As used throughout this specification and claims the term pliable plastic defines a viscous semi-solid mass of such a consistency that it is deformable under its own weight, but is not a free running mass as is the case in liquids. This defined mass is intermediate between a solid and a liquid, and will include some of the properties of, each, a liquid and a solid, but not all of either. The

meaning of the term semi-molten, hereinafter, is restricted to define a two temperature zoned mass of metal consisting of a pliable plastic core within a liquid surface layer. The pliable plastic core of the metal, as defined above, is at a temperature below the liquefying temperature of the metal whereas the liquid surface layer of the two zone mass of metal is at a temperature at or above the liquefying temperature of the metal. In addition, the term liquid suspension hereinafter refers to a two-phase system consisting of a finely divided solid dispersed in liquid. The term pellets as used hereinafter defines a substantial ellipsoid or special shaped smooth mass of metal.

The invention comprehends a method of fabricating metal pellets which eliminates the need for tall dropping towers and which provides substantially spherical pellets of consistent composition, devoid of air pockets and having a relatively smooth and clean surface. The weight of the individual metal spheroids thus produced is highly consistent. The invention contemplates dropping globules of metal in the semi-molten stage from an orifice and permitting the globule to fall 12 inches or less and preferably about 2 to 4 inches through air or other gas and into liquid suspension.

Figure 1 shows one method of obtaining metal in the pliable plastic condition. A metal 2 is melted in a crucible 4 and then cooled to the pliable plastic condition by being stirred with rods 6 of the same metal until the molten metal no longer rapidly melts the rods. The pliable plastic metal 8 is then poured into a second crucible 10 which is heated to maintain the metal in the pliable plastic condition. The heat input into the crucible is controlled to provide a thin liquid zone 16 along the walls of the crucible 10 to serve as a lubricant for the passage of the pliable plastic mass of metal through its passage in the crucible.

The second crucible has a discharge orifice 12 in its bottom wall. This pliable plastic mass of metal 8 will pass through the orifice 12 by gravity. By maintaining proper control of the temperature at the orifice 12 slightly above the melting point of the metal, the surface of the portion of the mass of pliable plastic metal in contact with the walls of the orifice, melts as indicated by 25, and acts as a lubricant for the remaining portion of the pliable plastic mass of metal to pass through the orifice as a semi-molten embryo globules 14.

It is necessary that the pliable plastic mass of metal pass from the crucible in a relatively short time to prevent the entire mass of semi-molten metal from being melted by the crucible or to prevent the temperature of the crucible from being lowered by the pliable plastic mass of metal to a point where it will no longer melt the contacting surface of the contained mass. The crucible temperature must be high enough to liquefy only the surface of the pliable plastic metal at the orifice but not so high that it will liquefy any appreciable amount of the mass contained in the crucible before the metal can pass through the orifice.

A suspension 18 is contained in a receptacle 20 with the top surface 22 of the suspension positioned about 12 inches or less below the bottom of the orifice 12. As the globules 14 of semi-molten metal emerge from the orifice and break off they fall through a resultant column of air or other gas and into the suspension 18 forming substantially spherical metal shot 24 having a substantially consistent composition throughout. Pellets produced by this method normally have a weight variation of only 10-15%.

Any liquid suspension which will withstand the temperature of the globules and has sufficient cooling capacity will produce satisfactory pellets. However, even suspensions which will decompose at the temperature of the globules will usually produce a few units of satisfactory pellets. For example, when aluminum in the semi-molten stage is dropped into a starch suspension in

water a few satisfactory pellets were obtained but as additional globules were dropped into the suspension the starch scorched. The resultant pellets ceased to be spherical and assumed a solidified configuration which resembled popped popcorn.

Various additives may be included in the suspension. For example, with colloidal graphite suspensions stabilizers such as ammonium hydroxide are generally required and with many suspensions it is desirable that soluble oils or salts be added to prevent the dispersed particles in the suspension from adhering to the newly formed shot. For example, the addition of 1% to 5% soluble oil or 10% common table salt added to a colloidal graphite suspension produced cleaner shot but had no other pronounced effect on the shot.

There is a definite relationship between the size of the orifice 12 and the consistency or fluidity of the suspension 18 for each different metal or alloy 8 being treated. The relationship adheres substantially to the rule that as the size of the orifice increases the consistency or fluidity of the suspension must be decreased. Of course, as the size of the orifice increases the size of the resultant pellets also increases and optimum ranges exist for each different combination of metal or alloy, orificed size and the consistency or fluidity of the suspension.

For example, the following table lists for different metals 8, the size of pellets 24 produced for various diameters of the orifice 12 as well as the percentage of colloidal graphite in the water suspension 18. The globules were dropped through a 2 to 4 inch column of air. It should be noted that smaller pellets can be produced when the semi-molten globule of metal is dropped from an orifice smaller than  $\frac{1}{16}$ " if a sufficiently high hydrostatic head is applied to force the pliable plastic metal through the orifice. The pellets are substantially spherical but may flatten slightly depending on the precise percentage of dispersed matter in suspension. In the event that the pellets are not absolutely spherical the following table indicates the largest diameter.

| Metal         | Pellet Diameter (inches) | Pellet Weight (grams) | Orifice Diameter (inches) | Percent by Weight Colloidal Graphite in Water |
|---------------|--------------------------|-----------------------|---------------------------|-----------------------------------------------|
| Aluminum..... | 0.700                    | 7.0                   | $\frac{1}{16}$            | 10-15                                         |
|               | 0.375                    | 1.10                  | $\frac{3}{16}$            | 12-15                                         |
|               | 0.300                    | 0.60                  | $\frac{3}{16}$            | 15-18                                         |
| Nickel.....   | 0.275                    | 0.40                  | $\frac{1}{16}$            | 18-21                                         |
|               | 0.110                    | 0.15                  | $\frac{5}{64}$            | 21                                            |
| Copper.....   | 0.100                    | 0.13                  | $\frac{1}{16}$            | 21                                            |
|               | 0.090                    | 0.15                  | $\frac{5}{64}$            | 21                                            |
|               |                          | 0.12                  | $\frac{1}{16}$            | 21                                            |

In addition to the above listed metals a 5 to 30 mix brass, phosphorous and silicon bronzes and cupro nickel have been satisfactorily formed into pellets by this process. Lead pellets formed by dropping in a 100 foot high dropping tower have a diameter ranging from about 0.005 inch to 0.180 inch. Substantially spherical pellets of aluminum and silicon bronze larger than  $\frac{1}{2}$  inch have been readily formed by the instant process.

In making pellets of commercially pure aluminum (1100 or 2S alloy), which contains a minimum of 99.0% chemically pure aluminum, the aluminum is melted and then cooled to the pliable plastic condition at a temperature range between 643° C. and 657° C. and preferably 650° C.  $\pm$  2° C., as previously described. The pliable plastic mass of aluminum is then transferred to a second crucible preheated to between 675-750° C. and having an  $\frac{1}{8}$  inch orifice in its bottom wall. The aluminum passes through the orifice as above described, and drops through air a distance between 2 to 4 inches into a water suspension of the type indicated in the following table.

The following table indicates the preferred percentage of material suspended in water. These percentages may

vary a small amount depending on the grain size of the suspended material.

| Suspended material:                 | Percent by weight of material suspended in water |
|-------------------------------------|--------------------------------------------------|
| Bentonite                           | 8-12                                             |
| Fuller's earth                      | 20                                               |
| Pax hand cleaner                    | 22-30                                            |
| Cupolo patch                        | 80 (approx.)                                     |
| Talc                                | 46                                               |
| Sodium alginate                     | 1-3                                              |
| Sodium alginate plus 1% soluble oil | 1.5-2.5                                          |
| Sodium alginate plus 5% soluble oil | 1.5-2.5                                          |
| Jaguar gum                          | 1.5-2.0                                          |
| Jaguar gum plus 1% soluble oil      | 1.2-1.8                                          |
| Bone ash                            | 56-62                                            |
| Diatomaceous earth (Silocel)        | 27-29                                            |
| Colloidal graphite (in Prodag)      | 12-15                                            |
| Graphite                            | 20                                               |

Various materials well known in the art may be added to the suspension to increase the suspendability of the dispersed matter.

Any suitable colloidal graphite may be used such as that available under the trade name "Superflake" manufactured by Superior Graphite Co., Chicago, Illinois, or "Prodag" manufactured by Acheson Colloids Co., Port Huron, Michigan. It has been found that a suspension of colloidal graphite produces satisfactory results when held between temperatures of 35-100° F. and preferably between 38-80° F. The temperature of the suspension must be high enough to prevent the liquid from freezing but low enough so that the globules of semi-molten metal will solidify very rapidly. Also, colloidal graphite is generally provided with a stabilizer such as ammonium hydroxide and when using this material it is necessary that the bath temperature be kept below about 100° F. so that the stabilizer will not be driven out of the suspension. The following suspensions in water: 43-45% starch, 10% stearic acid and 2% caustic solution, or 1% agar agar each produced a few satisfactory pellets but subsequent pellets were of nondescript configuration because the starch was scorched, and the stearic acid and agar agar was melted by the temperature of the globules. Accordingly, any particulate solid inert at the temperatures to which the bath is subjected is suitable as a material to be dispersed in a liquid in forming the suspension so long as the particles are sufficiently small and present in the correct amount.

It is to be understood that the invention is not to be limited to the specific suspensions enumerated in the description of the invention nor is the invention to be limited to the particular method of obtaining metal in the pliable plastic stage, and the semi-molten globules as herein described and as set forth in appended claims. Although several specific embodiments, materials and details have been set forth in the foregoing description it will be understood that various changes may be made without departing from the spirit and scope of this invention and that this invention is therefore not to be limited to such specific embodiments, materials or details except as set forth in the appended claims.

I claim:

1. The process of fabricating metal pellets which comprises maintaining a mass of metal in a pliable plastic state, separating a portion of the metal from said mass in a quantity sufficient to form a globule of said metal, heating the said separating portion of metal to an extent sufficient to liquefy the surface thereof and form a liquid layer on the core of the separated globule but insufficient to affect the physical state of the core within the globule, and cooling said globule by dropping it into a liquid suspension said liquid suspension being stable at the temperature of the globule upon entry thereto, and said cooling being sufficient to cause solidification of said globule.

2. The method of forming metal pellets comprising providing a mass of metal in a plastic, pliable state, separating and simultaneously heating a portion of said metal to an extent sufficient to form globules of said metal consisting of a pliable plastic core of metal within a completely liquefied surface layer, and cooling said globules by dropping them into a liquid suspension which is stable at the temperature of the globules upon entry into the suspension, said cooling being sufficient to cause solidification of said globules.
3. In a process of fabricating metal shot by passing the metal through an orifice to form a globule and cooling the metal by dropping it through a fluid bath, the improvement comprising passing said metal through said orifice while said metal is in a pliable plastic condition, completely liquefying the surface of a portion of said metal to form a globule and cooling said globule by passing it through a liquid suspension which is stable at the temperature of the said globule upon entry into the suspension, said cooling being sufficient to cause solidification of said globules.
4. The process of forming metal pellets comprising passing metal in a pliable plastic condition through an orifice completely liquefying the surface of a portion of said metal in its passage through said orifice to form globules and cooling said globules by dropping them into a liquid suspension which is stable at the temperature of the globule upon entry into the suspension, said cooling being sufficient to cause solidification of said globules.
5. The method of forming metal pellets comprising forming globules of metal with the metal temperature being in the range wherein the globule consists of a core in a pliable plastic condition within a completely liquefied surface layer and cooling said globules by dropping them into a suspension which is stable with the temperature of the globules upon entry into the suspension, said cooling being sufficient to completely solidify said globules.
6. The method of forming metal pellets comprising forming globules of metal at a temperature wherein the core of the said globule is in a pliable plastic condition, and said core is within a completely liquefied surface layer and cooling said globules by dropping them into a suspension which is stable at the temperature of the globule upon entry into the suspension, said cooling being sufficient to cause solidification of said globules.
7. The method of forming a metal pellet comprising melting a mass of metal to form molten metal, cooling the molten metal to below the melting point wherein said metal is in a pliable plastic condition, liquefying the surface of a portion of said metal to form a globule and solidifying said globule by dropping it into a liquid suspension which is stable at the temperature of the globule upon entry into the suspension.
8. The method of claim 7 wherein said molten metal is cooled by stirring the molten metal with a solid mass of metal until the molten metal no longer rapidly melts the solid mass.
9. The method of claim 8 wherein the solid mass of metal is of the same composition as the molten metal.
10. The method of claim 7 wherein the metal is melted and cooled in a first crucible and wherein the cooled metal is then poured into a second crucible at a temperature slightly above the melting point of the metal.
11. The method of claim 10 wherein the metal in a pliable plastic condition is passed through an orifice in said second crucible wherein the surface of a portion of said metal is completely liquefied to form a globule and said globule is dropped into said suspension.
12. The method of claim 11 wherein upon emerging from said orifice the said globule of metal drops a maximum distance of about 12 inches before entering said suspension.
13. The method of forming metal pellets comprising passing flowable metal in a pliable plastic condition

through an orifice, liquefying the surface of a portion of said metal in said orifice to form a globule, and cooling said globule by dropping it into a liquid suspension which is stable at the temperature of the globule upon entry into the suspension, said cooling being sufficient to solidify said globule.

14. The method of claim 13 wherein the metal is aluminum.

15. The method of claim 13 wherein the metal is nickel.

16. The method of claim 13 wherein the metal is copper.

17. The method of claim 13 wherein the suspension comprises a dispersion of colloidal graphite.

5 References Cited in the file of this patent

UNITED STATES PATENTS

|              |          |               |
|--------------|----------|---------------|
| 496,044      | Deniston | Apr. 25, 1893 |
| 1,903,329    | Beard    | Apr. 4, 1933  |
| 1,932,499    | Woods    | Oct. 31, 1933 |
| 10 2,403,463 | Seliger  | July 9, 1946  |
| 2,712,621    | North    | July 5, 1955  |